

Patented Sept. 5, 1922.

1,427,844

# UNITED STATES PATENT OFFICE.

HENRY ROBERT POWER, OF NIAGARA FALLS, NEW YORK, ASSIGNOR TO THE CARBO-RUNDUM COMPANY, OF NIAGARA FALLS, NEW YORK, A CORPORATION OF PENNSYLVANIA.

## ABRASIVE ARTICLE.

No Drawing.

Application filed November 17, 1919. Serial No. 338,604.

*To all whom it may concern:*

Be it known that I, HENRY ROBERT POWER, a citizen of the United States, residing at Niagara Falls, in the county of Niagara and 5 State of New York, have invented a new and useful Improvement in Abrasive Articles, of which the following is a full, clear, and exact description.

The invention relates to abrasive articles 10 such as grinding wheels and the like, and more especially to such abrasive articles containing a resinous bond.

In making abrasive articles such as abrasive wheels of this character, abrasive grains 15 or particles such as silicon carbide, or aluminum abrasives such as emery, aloxite or corundum are held together by a bond containing shellac. In some such compositions the abrasive grains are mixed with powdered 20 shellac, with or without the addition of powdered rosin, and compounding chemicals and fillers. This mixture is warmed sufficiently to mold into shape, and afterwards is baked to convert the shellac into a hard 25 elastic bond which holds the abrasive grains securely in place. During the baking process the rosin reacts chemically with the compounding chemicals to form resinates which also have certain bonding properties. When 30 rosin is used in such abrasive mixtures, a chemically equivalent amount of a metallic oxide, such as zinc oxide, lead oxide or lime, is required to react with the rosin to form a resinate, the melting point of which is 35 higher than the original rosin. For example, rosin employed in compounding abrasive mixtures melts at about 60° centigrade, whereas the zinc, lead or calcium resinates or "driers" melt at a temperature 40 of from 115° to 145° centigrade.

As a substitute for such rosin or resinates I use a resinous coal-tar distillate. This resinous distillate is preferably a polymerized compound of the coumarone-indene 45 group. In making abrasive compositions I have used a compound of this character known commercially as "cumar," a mixture of polymerized benzofuran or paracoumarone and paraindene. This is obtained 50 from the distillation of coal-tar. When coal-tar is distilled, one of the distillates is known as "light oil," which on distillation yields among other things "heavy naphtha." This in turn yields on distillation compounds of 55 the coumarone-indene group, such as coum-

arone and indene, these substances being unpolymerized or polymerized depending upon the temperature control of the process. If uncontrolled, the process yields polymerized products. If the process is properly 60 controlled the products are substantially unpolymerized and may be later put through a polymerizing process which yields as the ultimate product the polymerized products such as paracoumarone and paraindene. 65 The substance known commercially as "cumar" is a mixture containing paracoumarone and paraindene. The substances, however, may be used alone. For example, substantially pure paracoumarone of the proper 70 grade may be used in place of the commercial mixture.

The term "coumarone resin," as used herein, is therefore intended to include not only substantially pure paracoumarone, but also 75 the resins known commercially as "coumarone resins" which contain other polymerizable compounds of the coumarone-indene group. In my Patent, No. 1,310,292, granted July 15, 1919, for abrasive wheel, I 80 have more fully defined the organic compounds referred to and given the structural formulæ therefor.

There are several commercial grades of 85 cumar or paracoumarone, some being highly refined and odorless, tasteless and almost odorless. Others have a characteristic light yellow to a dark brown color. The grades that are hard at ordinary temperatures are brittle. Others are tough and cold flowing 90 at ordinary temperatures. The melting points of the different grades vary from 50° centigrade to 160° centigrade. The specific gravity is about 1.1 in all grades. On heating, it melts, giving a pleasant sweetish odor 95 and on cooling again is found to have lost none of its former chemical and physical properties. It is practically inert; it has no saponification number, no acid number; it is insoluble in alcohol and dissolves readily 100 in solvent naphtha. With an alkali it yields no lather. Furthermore, it oxidizes very slowly, even in the presence of strong oxidizing agents like nitric acid.

The use of the above described compound 105 or compounds of the coumarone-indene group has distinct advantages in the manufacture of abrasive articles, particularly those in which a shellac or similar elastic binder is used.

When used as a substitute for the resinates or so-called driers, the higher melting grades of cumar or paracoumarone, such as those having the melting point at about 5 160° centigrade, are employed. The cumar thus used requires no equivalent amount of metallic oxide as does rosin, for it melts at a temperature equal to that of the substituted resinate. Furthermore, cumar is a 10 neutral substance and if it is used together with some rosin, it will not react with the basic oxides present in the abrasive mixture. The cumar can be used either as a complete substitute for rosin and metallic oxides 15 or it may be used with them. It permits a saving in the amounts of both the metallic oxide and rosin or metallic oxide alone.

Such a substitution also permits of a larger percentage of abrasive grains in the 20 mix, to the extent of the amount of metallic oxide eliminated from the mix by substituting its equivalent chemically in rosin with the cumar or paracoumarone. Therefore, this gives compositions of different grades 25 than are possible when the rosin-oxide mixes are used. On the other hand, if a lower abrasive grain content is desired, metallic oxide fillers may be used in place of the abrasive grains without influencing the 30 bonding properties of the binder because the cumar or paracoumarone remains inactive with respect to the basic oxides.

In addition to this use of cumar or paracoumarone which results in economy and 35 flexibility in the mixes, there is the difference in character of the bond produced with shellac and cumar as compared with shellac and rosin-oxide compositions. Cumar or paracoumarone is decidedly brittle and gives 40 a quick wearing composition which continually exposes fresh surfaces of abrasive

grains. It is not likely, therefore, to glaze or become filled with particles of the material abraded.

In making abrasive articles such as abrasive wheels, I mix the abrasive grains together with powdered shellac and the powdered cumar or paracoumarone, with or without powdered rosin and basic materials and fillers, and mold the mix either cold or 45 warm into the desired shape. The shaped article is then baked at a temperature sufficiently high to cause the bond to flow and hold together the abrasive grains, the particular temperature used for baking depending 50 upon the composition of the mix.

While I have specifically described the preferred embodiment of my invention, it is to be understood that the invention is not to be limited to all of the details hereinbefore described, but may be otherwise embodied within the scope of the following claims.

I claim:

1. An abrasive article comprising abrasive particles and a binder containing shellac and coumarone resin. 65
2. An abrasive article comprising abrasive particles and a binder containing shellac, rosin and coumarone resin. 70
3. An abrasive article comprising abrasive particles and a binder containing coumarone resin. 75
4. An abrasive article comprising abrasive particles and a binder containing a polymerized resinous coal-tar distillate.
5. An abrasive article comprising abrasive particles and a binder containing a resinous coal-tar distillate.

In testimony whereof, I have hereunto set 80 my hand.

HENRY ROBERT POWER.